

H. S. LUCAS.

Torpedo.

No 58656.

Patented Oct. 9. 1866



Witnesses.

Jas. D. Patterson  
Thomas C. Smith, Attorney for Plaintiff  
Herman S. Lucas by *John L. Hayes*  
*Attorney*

Inventor.

# UNITED STATES PATENT OFFICE

HEMAN S. LUCAS, OF CHESTER, MASSACHUSETTS.

## IMPROVED BLASTING-CARTRIDGE.

Specification forming part of Letters Patent No. 58,656, dated October 9, 1863.

*To all whom it may concern:*

Be it known that I, HEMAN S. LUCAS, of Chester, in the county of Hampden and State of Massachusetts, have invented a new and Improved Cartridge for blasting purposes; and I do hereby declare that the following is a full and exact description thereof, reference being had to the letters and drawings forming a part of this specification.

The nature of my invention consists in forming a cartridge for blasting purposes of a cylinder of solidly-compressed gunpowder, or of any other explosive materials capable of being safely compressed into a suitable form, with suitable perforations or other appliances for igniting, and so protected and covered as to be impermeable to water.

To enable others skilled in the arts to use my invention, I will now proceed to describe its construction and operation.

To form the cartridge I take a hollow cylinder, either of metal or of wood, preferring metal, made slightly tapering, so as to facilitate the drawing of the cartridge when made. I fix in the center of this cylinder a slightly conical pin of metal, to form a central cavity in or perforation through the compressed powder. I have a rammer, made of hard wood or metal, preferring bronze, with a hole to fit upon the central pin and to exactly fill the cylinder. I fill this hollow cylinder with meal or other form of gunpowder, using either nitrate-of-potash or nitrate-of-soda powder, (the latter being preferred on account of its cheapness and equal efficiency,) or any other kind of explosive material capable of being slightly compressed. Having first slightly dampened it, I compress this powder into a very solid or stone-like mass, either by driving down the powder little by little by means of a mallet striking upon the driver, or by means of a screw or a hydraulic press, preferring the latter as most effective. When I have compressed my powder into a solid substance and form, as above described, I remove it from the cylinder. It is now a cylindrical or slightly conical mass of gunpowder with a central hole running through it from end to end.

I desire to observe that I have described the mode of constructing the solid cartridge and the form which I have found most con-

venient. I do not limit myself, however, to the mode above described of forming the solid cylindrical cartridge, nor do I limit myself to the cylindrical form of the solid cartridge, as other modes of constructing the solid cylindrical cartridges and other forms of solid cartridges may be found more convenient or useful. Neither do I limit myself to solid cartridges with perforations extending wholly through the center, as I sometimes use solid cartridges with perforations extending partly through the center, and the central perforation may be wholly dispensed with when other modes of igniting the solid cartridge at the center are used, as may be done by conducting an electrical current by means of a wire or otherwise.

When the cylinder of solid powder is formed as above described, and thoroughly dried, I take the cylinder and wrap it carefully with tough, well-made, and varnished paper, impermeable to water, sealing up the cylinder of powder in it, covering that which is to be the lower end entirely, and leaving proper projections beyond the end which is to be uppermost for attachment of the fuse when the charge is to be put into the blast-hole. (Gun-paper or gun-cloth cemented with collodion may be used as envelopes for the solid powder; but I do not employ these materials on account of their greater expense, preferring simple varnished paper or cloth.) A few grains of granulated powder may be first put into the cavity, and then the fuse may be affixed by inserting it into the hole in the middle of the cartridge; or this powder may be omitted, if desirable, as the fuse itself will fire the solid powder. The paper in excess beyond the cartridge is drawn around the fuse and tied tightly by means of twine. No cement is required unless the cartridge is to remain for a long time in a wet hole. In such a case a little wax or pitch may be put around the fuse when the paper is tied. The cartridge is now ready to be put in the drilled hole in the rock, and may be tamped in the usual manner.

I have described the mode of enveloping the solid cartridge which I prefer on account of its cheapness and simplicity. Other envelopes or cases for the solid cartridge may be used, such as casings of sheet metal, earthen-

ware, or wood. Such casings may be applied to the solid cartridge after it is formed, or the powder may be compressed solidly into such cases and suffered to remain.

The accompanying drawings exhibit the cylinder of compressed powder as above described, with the perforation and the mode of attaching the paper covering and fuse.

Figure 1 is a section of the cylinder of compressed powder. The solid compressed powder of the cylinder is represented at letter A. The central perforation is represented at letter B. Fig. 2 is a perspective view of the cylinder of compressed powder, with the paper covering and fuse attached. The paper covering is represented at letters A A A, the projecting portions of paper as tied at B B, the twine tying the paper to the fuse at C, and the fuse at D.

I will now proceed to present the advantages which the solid compressed cartridge for blasting, as above described, possesses above all others now known to miners, and the manner in which it acts in blasting.

First. It is safe from accidental firing, either when out of the drill-hole or in it, no loose powder being exposed to firing from any cause, either in the box containing the cartridges, or in the drill-hole, or around it.

Second. The charge may be drilled out with perfect safety, since no powder is exposed to sparks from the drill in removing the tampon.

Third. It may be used in holes above as well as below, or at any angle where loose powder could not be used, and where the clumsy, tarred, or greased pouches or bags are now commonly employed, which bags are made with great inconvenience, and at no small danger to the miner.

Fourth. This charge may be used in a wet hole without the least difficulty.

Fifth. Nitrate-of-soda powder (which is the cheapest) can be used in this solidly-compressed state without danger of deliquescence.

Sixth. The solid powder being fired in its center, has immense expansive force without that violent detonating initial action which is

so apt to blow out the tampon and only limited portions of rock around the hole. The solid powder, acting with continuous force, operates with more efficiency to overcome the elasticity of the rock than a sudden detonation.

I am aware that compressed gunpowder—sometimes, but incorrectly, called solid powder—has been used in firing heavy ordnance; but such powder consists in fact of large grains, and is used for a purpose directly opposite to that for which my solid charge is used, viz., to prevent the bursting of the gun. I do not claim the use of powder for blasting in large and separate grains.

What I claim as my invention, and desire to secure by Letters Patent, is—

1. A cartridge for blasting made of solidly-compressed gunpowder, containing either nitrate of potash or nitrate of soda, or granulated, or of any other suitable explosive material capable of being safely compressed into a suitable form for blasting purposes, and provided with any suitable device for igniting the same from the interior.

2. The combination of a cylindrical cartridge of solidly-compressed gunpowder, or other explosive materials, for blasting with a central perforation extending partly or wholly through the same, constructed in the manner and for the purpose above described.

3. The combination of a cartridge of solidly-compressed gunpowder, or other explosive materials for blasting with a fuse, when said fuse is inserted into its interior in the manner and for the purpose set forth.

4. The combination of a cartridge of solidly-compressed gunpowder for blasting purposes with an envelope of paper or other textile material made impermeable to water, or with envelopes or casings of sheet metal, earthen-ware, or wood, the same being attached to the fuse in the manner and for the purpose set forth.

HEMAN S. LUCAS.

Witnesses:

SAML. A. BARTHOLOMEW,  
ELIZABETH C. BARTHOLOMEW.